

Patented Jan. 17, 1939

2,144,532

## UNITED STATES PATENT OFFICE

2,144,532

## MANUFACTURE OF FOUNDRY MOLDS

John Howe Hall, Germantown, Pa., assignor to  
Birdsboro Steel Foundry and Machine Com-  
pany, Birdsboro, Pa., a corporation of Pennsyl-  
vania

No Drawing. Application February 12, 1933,  
Serial No. 396,323

4 Claims. (Cl. 22—189)

The present invention relates to the manufacture of foundry molds and, more especially, to an improvement in the process described in the Durand Patents Nos. 1,918,089, 1,918,090 and 1,924,028. As described in the Durand process, foundry molds are made of a mixture of sand and cement, with considerably less water than employed in usual cement-sand mixtures. This mixture is spoken of in the Durand patent as a "sub-hydrated" mixture. The water is so regulated that when the cement-sand mixture is taken in the hand, it is just coherent enough to form a highly friable ball. This mixture can be molded or tamped to form a mold or core of relatively high porosity and good structural strength. The Durand process has gone into rather extensive use and has made a distinct improvement in foundry practice. Difficulty, however, has been encountered in some instances, particularly in making castings of manganese steel and other metals poured at very high temperatures where the casting has re-entrant angles backed up by a considerable amount of metal, requiring a projecting part in the mold. The high heat of the metal and its access to both sides of the projecting part of the mold often results in the penetration of the sand by the metal, forming at the bottom of the re-entrant angle a porous mass consisting of a conglomerate of metal and partially fused sand which is exceedingly resistant to removal by cutting, grinding, or chipping. This action is apparently due to a combination of physical and chemical factors. The cement-sand mold mix must be porous to allow the escape of gases through the mold body. The sand, which is usually of silica or the like, under the high heat of the metal tends to fuse with the cement to form a sort of glass, which does not resist the penetration of the metal and tends to form the intensely hard conglomerate of metal and partially fused mold material. I have found that such disadvantages may be entirely overcome by providing a mold of the Durand type with a thin facing of substantial thickness composed of alumina bonded with cement. The alumina is preferably the fines of the fused alumina employed for abrasive purposes. This material is sold under various trade names, such as the well known trade-marks "Alundum" and "Aloxite". I have used the fused alumina fines passing a 200 mesh, with good results, in preferably approximately the following proportions:

|         | Parts |
|---------|-------|
| Alumina | 100   |
| Cement  | 13    |
| Water   | 7     |

While the water content may be somewhat more than that of the typical Durand mix, it is pref-

erable to use an amount of water substantially less than that employed in making the usual cement mixes, so that a mixture is formed which is moldable but which is not wet enough to slump and which will have a substantial porosity, although lower than that usually required by the Durand mixes.

In making a mold according to the present invention, a moldable mix of the aluminum oxide and cement is tamped against the pattern or core box to form a facing layer of about  $\frac{1}{2}$  to  $\frac{3}{4}$  of an inch thick. This facing layer may be employed over the entire face of the mold cavity, or may be employed only at the points where trouble would otherwise be encountered of the molten metal penetrating into the mold material. The term "facing" as used in the claim is intended to include a facing which may cover a part or the whole of the mold cavity. The surface of the facing which is away from the pattern is preferably left rough or roughened to provide a good bond with the cement-sand mixture which is next applied. The mold box or frame is then tamped full of the "sub-hydrated" mixture of sand and cement described in the Durand patents. The mold is preferably strengthened by iron rods embedded in the cement-sand mold material.

The mold box is taken off the mold, which is allowed to set as in the regular Durand process, and which is then ready for use.

The completed mold consists of a porous backing formed of the relatively dry or "sub-hydrated" mixture of sand and cement, and a highly refractory facing, which may be of considerably lower porosity and which is formed integral with the backing. The cement binder of the backing and facing unites the two parts together and there is little, if any, tendency for the facing to separate from the backing. The highly refractory character of the surface layer, and its higher density prevents the penetration of steel or other highly heated metal into the mold material. The backing, which is made of the regular Durand mix, has the high porosity required for the escape of the gases from the mold, and also has the structural strength required.

The highly refractory fused alumina resists the tendency to form a glass with the cement, which is encountered with the usual silica sands. While a limited amount of water is used to retain some porosity in the facing layer, the fine grain of the aluminum oxide fines gives a close grained structure to the facing which resists penetration of the metal and which gives a smooth surface to the casting.

While I prefer to use the fused alumina fines from abrasive manufacture, coarser grained alumina may be used if desired, although it is usually

more expensive and does not give as smooth a surface finish.

5 While the alumina is preferably the artificially formed fused alumina of the type used in abrasive manufacture, other forms of alumina may be used, for example, corundum, emery, or bauxite preferably calcined. The material should be granular to permit the requisite porosity.

10 While it is preferred that the facing layer be bonded with and supported by a cement bonded porous backing material like that specifically described in the Durand patents, other backing materials may be used, particularly in the making of cores where low resistance to collapsing is desired. In such case, the ordinary cement-sand mixture may be replaced in part or in whole by green or dry sand, cinders, or the like.

15 The facing layer consists principally of the alumina and may, if desired, contain minor amounts of other sands, but not sufficient however to materially affect the refractory properties of the mixture.

20 The material used for a binder is preferably high early strength Portland cement, although ordinary Portland cement or alumina cements 25 may be used.

25 The term "foundry mold" as used in the claims is intended to include cores as well as molds.

30 While I have described a preferred embodiment of my invention and have described par-

ticular materials which may be utilized it will be understood that my invention may be practiced or otherwise embodied within the scope of the appended claims.

I claim:

1. A foundry mold comprising a porous facing of substantial thickness composed principally of finely divided fused aluminum oxide bonded with cement, and a backing integrally united with the facing and composed principally of ordinary sand 10 bonded with cement and having a high porosity.

2. A foundry mold comprising a facing of substantial thickness composed principally of granular refractory aluminum oxide bonded with cement, and a porous backing composed principally of sand and cement integrally united with the facing. 15

3. A foundry mold comprising a facing formed from a moldable but friable mix consisting principally of granular alumina and cement together 20 with an amount of water insufficient to form a dense mixture, and a backing formed from a moldable but friable mixture of sand and cement containing so little water as to form a mass of 25 high porosity.

4. A foundry mold having a facing consisting principally of granular refractory alumina bonded with cement. 30

JOHN HOWE HALL. 30